

# United States Patent Office

3,545,973

Patented Dec. 8, 1970

1

## 3,545,973 PHOTOSENSITIVE POLYVINYLBUTYRAL LACQUER

Theo Tjalke Boersma, Hendrik Johannes Veenendaal, and Hendrikus Cornelis Nicolaas van der Sanden, Em-masingel, Eindhoven, Netherlands, assignors, by mesne assignments, to U.S. Philips Corporation, New York, N.Y., a corporation of Delaware

No Drawing. Filed Apr. 18, 1967, Ser. No. 631,578  
Claims priority, application Netherlands, Apr. 20, 1966,

6605244

Int. Cl. G03c 1/66

U.S. Cl. 96—93

2 Claims

### ABSTRACT OF THE DISCLOSURE

Photosensitive materials comprising a polyvinylbutyral lacquer and an aliphatic alkaryl, dimethyl ammonium bichromate. An example is dimethyllaurylbenzyl ammonium bichromate.

The invention relates to the preparation of a photosensitive polyvinylbutyral lacquer which contains a water-insoluble polyvinylbutyral resin and a bichromate. Such lacquers are used in photomechanical processes.

In the applicants' prior patent application, application Ser. No. 498,144, filed Oct. 19, 1965, now Pat. No. 3,471,294, it is stated that photosensitive lacquer of this type may particularly advantageously be prepared by using a water-insoluble or substantially water insoluble organic bichromate which, however, is readily soluble in solvents in which the polyvinylbutyral resin is soluble.

When using these organic bichromates it was found that the dark reaction in lacquer layers on a metal substrate proceeds off more slowly than in lacquers which contain inorganic bichromates.

It has been found that the physical and photomechanical properties of the resulting lacquer layers also are less influenced by the climatological conditions existing while drying the layers.

Thermally stable lacquers, that is to say, lacquers having long pot lives, are obtained in particular with organic quaternary ammonium bichromates of the general formula:



in which  $n=0, 1, 2$  or  $3$ . According to said prior patent application, R may be an aliphatic saturated or unsaturated hydrocarbon chain having 6 to 18 carbon atoms or an alicyclic ring. If  $n$  is smaller than 3, the various hydrocarbon radicals R may be different or the same.

Examples of such compounds are dimethyllauryl ammonium bichromate and trimethyllauryl ammonium bichromate.

According to the invention, it has been found that improved results are achieved by the use of quaternary ammonium bichromates of the formula:



wherein  $R_1$  is an aliphatic hydrocarbon moiety of 6-18 carbon atoms inclusive and  $R_2$  is alkaryl of 7 to 12 carbon atoms inclusive.

It has been found that these compounds are more soluble in the solvents for the polyvinylbutyrals than the corresponding quaternary ammonium bichromates of the prior application. Thus by use of the bichromates of the instant case, it is possible to produce lacquers of higher sensitivity.

In the bichromates of this invention  $R_1$  may be for example, octyl, decyl, dodecyl (lauryl), tetradecyl (myristyl) hexadecyl (cetyl), octadecyl (stearyl).

2

$R_2$  may be benzyl, ethylbenzyl and naphtylmethyl. Specific examples are: dimethyllaurylbenzylammonium bichromate, dimethylmyristylbenzylammonium bichromate, dimethyllaurylethylbenzyl ammonium bichromate, dimethylcetyl benzylammonium bichromate, dimethylcetyl ethylbenzylammonium bichromate.

The differences in solubility are shown in the following table which relates to a polyvinylbutyral lacquer employing as a solvent a mixture of 62% by volume of methylisobutylketone and 38% by volume of dimethylformamide in which the solubility of various bichromates was determined.

Solubility at 20° C.  
in g. per 100 ml.  
of lacquer

|    |                               |             |
|----|-------------------------------|-------------|
| 15 | Bichromate:                   |             |
|    | Trimethyllauryl ammonium      | 3           |
|    | Dimethyllauryl ammonium       | 5           |
|    | Dimethyllaurylbenzyl ammonium | exceeding 5 |

20 The preparation and the use of a lacquer according to the invention will now be described in greater detail with reference to the following example.

### EXAMPLE

25 4 g. of dimethyllaurylbenzyl ammonium bichromate was added to a solution of 13 g. of polyvinylbutyral (vinyl alcohol content approximately 20% by weight, viscosity of a standard solution of 10% by weight of polyvinylbutyral in 95% methanol: 120 cm. at 25°) in a mixture of 75 mls. of dimethylformamide and 125 mls. of butane. After the complete dissolution of the bichromate, a previously cleaned copper plate was dipped in this solution in such manner that after drying in air of 40° C. an evenly thick lacquer layer was obtained. This layer was exposed to light through a template for 1 minute by means of four 125 watt high pressure mercury discharge lamps placed in the corners of a square having sides of 15 cms. at a distance of 50 cms. from the object. The unexposed parts of the lacquers were then washed away in methanol. The remaining lacquer pattern may be used as a screening layer for various etching or electro-deposition processes.

30 While we have described our invention in connection with specific embodiments and applications, other modifications thereof will be readily apparent to those skilled in this art without departing from the spirit and scope of the invention as defined in the appended claims.

What we claim is:

35 1. A photosensitive polyvinylbutyral lacquer containing a water-insoluble polyvinylbutyral resin and an organic quaternary ammoniumbichromate of the formula:



40 55 wherein  $R_1$  is an aliphatic hydrocarbon chain of 6 to 18 carbon atoms and  $R_2$  is aralkyl of 7 to 12 carbon atoms.

2. The photosensitive lacquer of claim 1, wherein dimethyllaurylbenzylbichromate is employed.

### References Cited

#### UNITED STATES PATENTS

3,471,294 10/1969 Boersma et al. 96—93

#### FOREIGN PATENTS

1,123,642 8/1968 Great Britain 96—93

RONALD H. SMITH, Primary Examiner

U.S. Cl. X.R.

96—36, 75, 115